

## UNITED STATES PATENT OFFICE

1,987,195

## PROCESS FOR THE DIGESTION OF VEGETABLE GROWTHS TO PRODUCE CELLULOSE

Herman B. Kipper, Accord, Mass.

No Drawing. Application March 3, 1934,  
Serial No. 713,856

6 Claims. (Cl. 92—9)

In my Patent Number 1,820,276 of August 25, 1931 I described processing for digestion of vegetable growths and more especially wood for production of cellulose and more especially paper pulp. According to the processing described in the above patent mechanical disintegration of the wood is established simultaneously with chemical disintegration or digestion by means of bevelled bars or knives which travel with cylindrical motion within the digester and through the digestion mass at a high rate of speed. Reductions in the chemicals required and in the time and temperature of digestion are thereby established. In my copending applications Serial Nos. 660,649 of March 14, 1933, 665,957 of April 13, 1933, 682,942 of July 31, 1933 and 689,875 of September 18, 1933, I describe specific improvements in digestion media as applied to my basic method of processing.

My present invention embodies a further improvement over the above processing for digestion of vegetable growths for recovery of cellulose. Such improvement depends more especially on a further reduction in the temperature required for digestion and hence positive further reduction in the fuel requirement. In order to accomplish this latter result air or oxygen is passed into the digester and through the digestion liquid or mass. Such air or oxygen may be passed into the digester at the bottom of the same, or through a perforated hollow shaft bearing the disintegration bars or knives, or again in any other suitable manner, as at the ends of my horizontal digester. I have used satisfactorily all three methods mentioned. When employing this method of digestion I have found it necessary to employ only a hot aqueous solution of the digestion chemicals and air or oxygen at atmospheric or superatmospheric pressure. In other words, the digestion solution need not be heated above its boiling point. This method of digestion I have found especially advantageous for use in the recovery of the cellulose fibre from waste cotton seed hulls.

In digestion of these waste hulls from their cellulose content I used a small digester two feet long by sixteen inches internal diameter. A quarter inch pipe coil was wound externally around the digester and used for heating the latter with steam. For large scale operation such external heating should be practically unnecessary as the ratio of surface to cubical contents in the latter case would be greatly reduced and hence surface radiation of heat correspondingly lessened. Insulation might be required. The

above digester was partially filled with some twenty pounds of waste cotton seed hulls and a hot aqueous solution containing from five to fifteen percent of sodium hydroxide on the weight of waste hulls was run into the same until about three-fourths filled. The beater blades traveling at about a speed of twenty feet per second and nine hundred revolutions per minute were then started and oxygen forced into the bottom of the digester at a rate of about ten cubic feet per hour. Digestion was continued for seven hours. The pulp was then removed, the digestion liquor drawn off from the pulp by means of a suction filter and the pulp suitably washed. A good pulp high in alpha-cellulose was secured. The spent digestion liquor, of course, can be evaporated for recovery of chemicals or again it may be evaporated to dryness. A plastic material is secured by the latter step which is adaptable for moulding purposes.

I have also employed oxygen at a superatmospheric pressure and up to fifty pounds and at eighty-five to one hundred degrees centigrade for digestions otherwise similar to that just described. The digestion period is thereby materially reduced. The same was completed within about an hour. I also used air in place of oxygen in a digestion practically the same as those already described with the exception that about five times the volume of air was used instead of the oxygen as already noted and the pressure was maintained at about one hundred pounds. The oxygen or air might, of course, be circulated through the digester by a pump situated externally.

Furthermore, for the digestion agents I have used calcium hydroxide, ten to fifteen percent on the weight of hulls suspended in the digestion mass, and calcium hydroxide in conjunction with sodium chloride, from one to five percent, in solution. Calcium hydroxide is of course, only very slightly soluble. Equilibrium between the sodium chloride and calcium hydroxide in solution occurs and a small percentage of sodium hydroxide is formed. As the latter is quickly utilized in the digestion process its regeneration with establishment of equilibrium is brought about, so that a small percentage of sodium hydroxide is constantly available for the digestion. The latter is far more active than the corresponding calcium hydroxide, but so-called hydrated lime is, of course, much the cheaper chemical so that its use is greatly to be preferred. Without the rapid mechanical mixing or disintegration employed in my type of digester the use of such lime, however, is impracticable and such

statement furthermore is very nearly pertinent to the use of oxygen or air for the digestions described. As the percentage of sodium hydroxide present in the solution at any given time, however, is small, the digestion period is considerably increased and six to eight hours were required. In order to establish the more rapid digestion and at the same time to reduce costs of operations I have further employed a solution of sodium-carbonate and calcium hydroxide suspended in solution. The reaction occurring between these two chemicals to form sodium hydroxide and calcium carbonate is very quickly brought about in the digester itself.

When using wood, cut into chips regularly used for pulp reduction, the above described methods of digestion are inoperative. The wood chips have to be pre-treated with oxygen or air and oxides of nitrogen, or nitric acid vapor, or soaked in an aqueous solution of ten to twenty percent nitric acid. Subsequent to such treatment, however, I have found that I could use hydrated lime or calcium hydroxide for fibre production also in conjunction with oxygen or air, in place of sodium hydroxide for final fibre liberation. The latter step is of great advantage because of the reduced cost of the calcium hydroxide, or hydrated lime, in comparison with that of the similar sodium salt.

The wood chips were first steamed to about a twenty percent moisture content and then treated for two to three hours with air at about fifteen pounds super-atmospheric pressure and with five to fifteen percent of the oxide of nitrogen and under constant mechanical beating as induced in my patented type of digester. The air supply was renewed continuously so that about ten to twenty percent of oxygen on the weight of wood was employed. Hot water containing ten to twenty percent, on the weight of wood, of calcium hydroxide in suspension was then run into the digester and beating continued for from one to two hours also under super-atmospheric pressure produced by air. In the latter case I used about fifty pounds pressure. It will be understood that the rapidly moving digestion mass is mechanically sprayed through the compressed air situated above it and hence forced penetration of the mass by oxygen continuously established. It is because of such action that I have been able to secure such efficient oxidation. The beater bars or knives in the digester travel at a speed of about twenty feet per second.

When using nitric acid in the vapor form the latter was diluted with forty percent of water and steamed into the digester. Otherwise the processing was practically that described.

When pretreating the wood with nitric acid about fifteen to twenty percent of the latter diluted with water was used, and the wood allowed to soak for some twenty-four to forty-eight hours depending on the size of the wood chips. It was then treated with air at about fifteen pounds superatmospheric pressure in my type of digester for an hour or two at fifty to one hundred degrees centigrade. The processing subsequently used was that already described. In the soaking process the percentage of nitric acid required is about double that needed in the first two mentioned methods so that the latter process is not relatively as efficient. I have used also a calcined dolomite stone in place of limestone, or a hydrate secured from the former. The pulp in such case is somewhat lighter in color. I have

further used sodium hydroxide in conjunction with calcium and magnesium hydroxide.

A limitless number of combinations of different chemicals in alkaline digestion liquors, in place of those described, might of course be employed. I used sodium nitrate and nitrite as well as sodium sulphite, and a combination of sodium nitrate and sodium sulphite in this connection, but without any very distinct advantages. Also other oxidizing agents as potassium permanganate and potassium dichromate were not found of sufficient added advantage to warrant the additional costs involved in their use. I have used only hot aqueous solutions of the digestion chemicals, as such were found entirely satisfactory, but, of course, higher temperatures and super-atmospheric steam pressures might be employed with consequent reduction in the digestion periods. On the other hand if colder digestion liquors are used we should expect to have to employ longer digestion periods. Although I have not used cold liquors I have employed the same heated only to fifty degrees centigrade and found such use as positive.

In freeing the cellulose from cotton seed hulls I have also used hydrated lime, or calcium hydroxide, in place of sodium hydroxide, or mixtures of these two chemicals, in conjunction with oxygen or air. For the latter step I employed about eighty per cent of lime, or the full equivalent of lime required and twenty per cent of sodium carbonate. Again I have brought about the digestion with sodium hydroxide, and after separation of the cellulose fibre from the spent hot digestion liquor I have treated the latter under stirring. The partially oxidized hull material is thereby precipitated as the calcium salt and the sodium hydroxide solution is regenerated for digestion purposes. The calcium salt of the oxidized hull material after drying, and while hot, is plastic and under pressure can be molded.

I have also used sodium and calcium hydroxides for wood digestion, but without oxygen, but even in my type of digester seventy five to one hundred pounds steam pressure are required.

I claim:

1. In a process for the digestion of vegetable growths to produce cellulose fibre and of disintegrating the said vegetable material mechanically by the action of cylindrically rapidly moving metal pieces which travel through the digestion mass simultaneously with the process of digestion by chemicals in aqueous solution the step of forcing oxygen (air) through the digestion mass simultaneously to the period of chemical digestion.

2. In a process for the digestion of vegetable growths to produce cellulose fibre and of disintegrating the said vegetable material mechanically by the action of cylindrically rapidly moving metal pieces which travel through the digestion mass simultaneously with the process of digestion by chemicals in aqueous solution the step of forcing oxygen (air) at superatmospheric pressure through the digestion mass simultaneously to the period of chemical digestion.

3. In a process for the digestion of vegetable growths to produce cellulose fibre and of disintegrating the said vegetable material mechanically by the action of cylindrically rapidly moving metal pieces which travel through the digestion mass simultaneously with the process of the digestion of the said vegetable matter by a hot aqueous solution of sodium hydroxide the step of forcing oxygen (air) at superatmospheric pres-

sure through the digestion mass simultaneously to the period of chemical digestion.

4. In a process for the digestion of vegetable growths to produce cellulose fibre and of disintegrating the said vegetable material mechanically by the action of cylindrically rapidly moving metal bars which travel through the digestion mass simultaneously to the said digestion process the step of digesting the vegetable matter by a hot aqueous solution of sodium hydroxide produced from sodium carbonate in the said solution and of calcium hydroxide suspended in the digestion mass and the step of forcing oxygen (air) at superatmospheric pressure through the digestion mass simultaneously to the period of chemical digestion.

5. In a process for the digestion of vegetable growths to produce cellulose fibre and of disintegrating the said vegetable material mechanically by the action of cylindrically rapidly moving metal bars which travel through the digestion mass simultaneously to the said digestion process the step of pretreating the vegetable matter with steam, oxygen, (air) and nitric oxides (nitric acid) and the step of digesting the said matter

with calcium hydroxide suspended in hot water and added to the digestion mass and finally the step of forcing oxygen (air) through the digestion mass simultaneously to the period of chemical digestion and by means of the rapidly traveling beater elements and with or without exterior circulation of the gas.

6. In a process for the digestion of vegetable growths to produce cellulose fibre and of disintegrating the said vegetable material mechanically by the action of cylindrically rapidly moving metal bars which travel through the digestion mass simultaneously to the said digestion process the step of pre-treating wood chips with steam, oxygen (air) and nitric oxides (nitric acid) at superatmospheric pressure and the step of digesting the said treated wood chips with calcium hydroxide suspended in hot water and added to the digestion mass and finally the step of forcing oxygen (air) at superatmospheric pressure through the digestion mass simultaneously to the period of chemical digestion and by means of the rapidly traveling beater elements and with or without exterior circulation.

HERMAN B. KIPPER. 25